

## UNITED STATES PATENT OFFICE

LELAND E. WEMPLE, OF CHICAGO, AND FLOYD A. WARREN, OF PERU, ILLINOIS, AS  
SIGNORS TO ILLINOIS ZINC COMPANY, OF CHICAGO, ILLINOIS, A CORPORATION OF  
ILLINOIS

## ZINC ALLOY

No Drawing.

Application filed October 18, 1929. Serial No. 400,724.

Our invention relates to new and useful alloys of zinc whose advantages will be hereinafter set forth. The alloys are prepared by adding to 100 parts of zinc from  $\frac{1}{4}$  to 2 parts of copper and a small proportion of silver. The alloys should be free from aluminum and magnesium, preferably completely, but in any event in proportions so substantial as to affect adversely their valuable characteristics.

The use of zinc, particularly when rolled into the form of sheets or strips, is limited because of its low tensile strength, its slight hardness, and the rapid dulling of its surface. These disadvantages are overcome if there be added to zinc both copper, in the proportion of  $\frac{1}{4}$  to 2% of the amount of zinc, and silver in the proportion of .1% to 20% of the copper. An alloy thus produced may be rolled into sheets and strips whose surface can be brought to an attractive condition by polishing, the polished surface maintaining its lustre, and which have a much higher tensile strength than sheets or strips rolled from zinc or known zinc base alloys. At the same time the natural advantages of the zinc are not reduced, in any event, to any appreciable or substantial extent. When used as a base metal for fixing etchings, the etching process can be carried out more rapidly than with ordinary zinc. The use of the silver toughens the alloy, and under some circumstances increases its ductility.

The zinc used in the production of the alloy may be a high grade zinc but for practical purposes we prefer to use the lower grades of commercial slab zinc or spelter which should, however, not contain ingredients which detrimentally affect the alloy. For instance the presence of more than .6% of cadmium or .04% of iron renders the zinc too brittle for rolling into thin gauges and the presence of over .6% of lead so decreases the tensile strength of the alloy that thin sheets rolled therefrom will tear even in the rolling process. The presence of even a small trace of aluminum causes the alloy, after rolling, to develop cracks and to disintegrate. For practical purposes we prefer to use a grade of spelter known in the trade as "intermedi-

ate," whose maximum iron content is .03%, maximum lead content .2%, and maximum cadmium content .5%, but not more than a total of .5% of all such metals, and which is substantially free from aluminum and magnesium. 55

We may, however, use to advantage the grade of spelter known as "brass special" or the grade known as "high grade."

The exact proportion of copper and of silver will depend upon the particular qualities of the alloy to be produced and also upon the various conditions of the process, for instance, rolling, to which the alloy is to be subjected. The particular proportions may easily be adjusted by simple experiment until the correct proportion suitable for the desired alloy is determined. 60 65

## Example

About 6 tons (12,000 pounds) of slab spelter—brass special—containing in addition to zinc iron .02% lead, .6%, and cadmium .08%, are charged into a coal fired tank furnace and the temperature of the furnace maintained at a temperature of 825° F. When the slabs are completely melted, forming a bath of molten zinc, i. e. after about six hours, the dross is carefully skimmed off and 30 pounds (or .25%) of copper in the form of wire are added and stirred into the molten metal. After the copper has been thoroughly incorporated with the zinc, 8½ ounces of silver (or 1.7% + relative to copper) are added in the form of pellets and stirred into the bath of molten metal. When both the copper and the silver are incorporated with the zinc, the molten alloy is cast into plates suitable for rolling. These plates after annealing in the manner usual with ordinary zinc i. e. by heating to 350°-400° C. are passed through roughing and finishing rolls, in the same manner as with ordinary zinc, to form sheets or strips. 75 80 85

It would be possible if desired to incorporate the silver first with the copper and to add the alloy thus produced, either in liquid or solid form, to the molten zinc. 90 95

The new alloy thus produced compares approximately as follows with ordinary rolled

1,789,854

zinc, provided both alloy and zinc were rolled  
in the same manner:

|                                  | New alloy                                  | Ordinary                   |
|----------------------------------|--------------------------------------------|----------------------------|
| 5 Hardness, Rockwell             | 97                                         | 87                         |
| Tensile strength<br>per sq. inch | 30,300 lbs.<br>42,300 lbs.                 | 25,000 lbs.<br>32,000 lbs. |
| 10 Dynamic ductility             | 350<br>Bends<br>with grain<br>across grain | 350<br>1½<br>1½            |

It will be noted that the hardness of our alloy is about 10 points greater by the Rockwell scale than ordinary rolled zinc and that the tensile strength of our alloy both with and across the grain is appreciably greater than that of ordinary zinc. At the same time the ductility of the alloy, as indicated by the readings on the dynamic testing machine and on the bending machine, shows that the increase in hardness and tensile strength has not been obtained at a sacrifice of ductility.

The alloy has a higher resistance in the electro-magnetic fields than ordinary zinc without having its ductility impaired, in any event, to any substantial degree.

Attention is called to the fact that these physical tests are significant only when compared with ordinary zinc rolled under identical conditions. The alloy of the example would, if rolled to a thinner gauge, have its tensile strength increased to 36,400 pounds, its dynamic ductility to 370, and its Rockwell hardness to 97½.

15 We claim:

1. As a composition of matter an alloy characterized by the fact that it is of substantially greater hardness than zinc composed of zinc 100 parts, copper  $\frac{1}{4}$  to 2 parts and an appreciable quantity of silver, such quantity being less than the amount of copper used.

2. As a composition of matter an alloy composed of zinc 100 parts, copper  $\frac{1}{4}$  to 2 parts and silver .1% to 20% of the copper.

3. As a new article of manufacture a mechanically worked zinc product made of a zinc base alloy composed of zinc 100 parts, copper  $\frac{1}{4}$  to 2 parts, and an appreciable quantity of silver, such quantity being less than the copper.

LELAND E. WEMPLE.  
FLOYD A. WARREN.